

## UNITED STATES PATENT OFFICE

2,221,258

## MAGNESIUM BASE ALLOY

John C. McDonald, Midland, Mich., assignor to  
The Dow Chemical Company, Midland, Mich., a  
corporation of Michigan

No Drawing. Application November 13, 1939,  
Serial No. 304,135

## 3 Claims. (Cl. 75—168)

The invention relates to magnesium base alloys. It more particularly concerns alloys of this nature having a high degree of formability, coupled with other improved physical properties, such as 5 high tensile and yield strengths.

Magnesium alloys are being widely used in various structural arts, where a light weight metal is highly desirable, such as for use in making castings, forgings, and the like. However, 10 the use of these metals in the rolled form to make sheet metal articles requiring forming operations, such as bending, drawing, and the like has not progressed as rapidly, due to the fact that in general alloys possessing good formability permitting relatively sharp bends to be made 15 without the article developing external cracks, usually have poor strength properties.

It is, accordingly, the principal object of the 20 invention to provide a magnesium base alloy which may be made into rolled sheet or the like, possessing a high degree of formability or ductility, permitting it to be sharply bent, drawn, or otherwise shaped while having improved strength characteristics.

25 Other objects and advantages will be apparent during the course of the following description of the invention.

My invention resides in the discovery that a 30 magnesium base alloy composed of from 0.3 to 10 per cent of silver, from 1 to 15 per cent of cadmium, from 0.1 to 3 per cent of manganese, and from 0.1 to 10 per cent of zinc, the balance being substantially all magnesium, is endowed with the afore-mentioned properties. While the property 35 of improved formability or ductility, associated with high tensile and yield strengths, is manifest over the entire range of composition indicated, I have found that, in general, the preferred combination of properties, such as the most desirable ductility for forming operations, coupled with high tensile strength and yield strength, is obtained when the alloy contains from 0.5 to 5 per cent of silver, 4 to 10 per cent of cadmium, 1.5 to 2.5 per cent of manganese, and from 0.5 to 5 per cent of zinc.

The specific proportion of each alloying metal and the total amount of the added metals to be employed in the new alloy depends upon the use for which the alloy is intended. In general, it is preferable to use an alloy containing more than about 75 per cent of magnesium and less than 25 per cent of the total added metal.

The following table, which lists some of the properties of rolled sheet metal made from my new alloy, as well as the properties of rolled sheet

of some of the related ternary alloys, illustrates the improvement in yield strength, tensile strength, and ductility of the new alloy over the corresponding properties of the closely related alloys. In the table the per cent elongation represents the ductility or formability of the alloys.

Table

| Nominal composition in percent (remainder=magnesium) |     |     |     | Annealed                       |                                  |                                | 10 |
|------------------------------------------------------|-----|-----|-----|--------------------------------|----------------------------------|--------------------------------|----|
| Ag                                                   | Cd  | Mn  | Zn  | Yield strength in lbs./sq. in. | Tensile strength in lbs./sq. in. | Percent elongation in 2 inches | 15 |
| 0.7                                                  | 5.0 | 1.8 | 0.8 | 27,000                         | 39,000                           | 15                             | 20 |
| 0.7                                                  | 2.0 | 1.0 | 0.8 | 27,000                         | 39,000                           | 16                             | 20 |
| 0.9                                                  | 5.0 | 0.9 | 1.0 | 18,000                         | 32,000                           | 20                             | 20 |
| 1.0                                                  | 5.7 | 1.5 | 0.8 | 28,000                         | 39,000                           | 17                             | 20 |
|                                                      | 4.6 | 1.5 | 4.0 | 27,000                         | 43,000                           | 15                             | 20 |
| 0.9                                                  | 2.2 | 3.5 | 4.0 | 25,000                         | 41,000                           | 16                             | 20 |
| 0.8                                                  | 5.1 | 4.7 | 4.7 | 17,000                         | 33,000                           | 20                             | 20 |
| 0.7                                                  | 5.6 | 1.0 | 4.8 | 26,000                         | 40,000                           | 18                             | 20 |
| 0.9                                                  | 5.7 | 1.5 | 4.8 | 29,000                         | 44,000                           | 16                             | 20 |

The properties listed in the above table under 25 the section headed by the term annealed were obtained by first rolling the alloys at a temperature between about 500° to 700° F., and thereafter annealing them at various temperatures through a 30 temperature range of from 400° to 800° F. The properties selected for the table were those of the annealed specimens which exhibited the maximum elongation.

By a comparison of the properties listed in the 35 above table it will be observed that the combined properties of my new polynary alloy are superior to those of the parent quaternary alloys having similar percentages of alloying ingredients. For example, it will be noted that the yield strength and tensile strength combined with the per cent 40 elongation, which serves as a measure of the ductility, shows improvement over that of the related alloys. In addition the alloys possess the characteristic of being highly resistant to corrosive 45 conditions.

While the new alloy is most useful in wrought form, such as sheets, due to its formability characteristics, it may also be suitably used in making castings, forgings, extruded forms, and the like. It is further pointed out that my new alloy 50 is amenable to solution and precipitation heat treatments, which, accordingly, modify its properties.

My new alloy may be prepared by any of the methods usually employed for melting and alloy- 55

ing metals with magnesium, such as by adding the respective metals singly or jointly to a bath of molten magnesium, which is preferably protected from oxidation by suitable flux.

5 1 claim:

1. A magnesium base alloy containing from 0.3 to 10 per cent of silver, from 1 to 15 per cent of cadmium, from 0.1 to 3 per cent of manganese, and from 0.1 to 10 per cent of zinc, the balance

10 being magnesium.

2. A magnesium base alloy containing from 0.5

to 5 per cent of silver, from 4 to 10 per cent of cadmium, from 1.5 to 2.5 per cent of manganese, and from 0.5 to 5 per cent of zinc, the balance being magnesium.

3. A magnesium base alloy containing from 1 to 5 4 per cent of silver, from 5 to 8 per cent of cadmium, from 1.5 to 2.5 per cent of manganese, and from 1 to 5 per cent of zinc, the balance being magnesium.

JOHN C. McDONALD. 10